

1

2,886,432

## ALUMINUM FOIL FOR ELECTROLYTIC CONDENSERS

Hans Schmitt, Rhinefelden, Baden, and Gustav Siebel and Dietrich Altenpohl, Singen am Hohentwiel, Germany, Hans Hug, Neuhausen am Rhinefall, Switzerland, and Johannes Nuesch, Mogliano Veneto, Italy, assignors to Aluminium-Industrie-Aktien-Gesellschaft, Chippis, Switzerland

No Drawing. Application November 15, 1956  
Serial No. 622,287

Claims priority, application Switzerland  
November 18, 1955

7 Claims. (Cl. 75—138)

Our present invention relates to an aluminum foil for electrolytic condensers, which foil has to be roughened by etching before the subsequent coating with an oxide or other dielectric film.

It is very difficult to etch satisfactorily aluminum foils of highest purity without use of electric current. Moreover, difficulties arise often during the electrolytic etching of high purity aluminum foils, which difficulties are caused for instance by the coarse grain structure of the metal.

A preferred, well known chemical etching bath consists in 6 to 10 percent hydrochloride acid with an addition of ferric chloride. For electrolytic etching, one uses for instance a solution of 1 percent sodium chloride in water.

It is known to add little quantities of chemical elements to the high purity aluminum in order to improve its ability to be etched. For instance, additions of 0.001 to 0.1 percent of lead, tin, bismuth, antimony, thallium, titanium, nickel, palladium, platinum, zirconium and other elements have been proposed. Amongst them, the addition of 0.01 to 0.03 percent boron has also been proposed.

Up to now, the proposed additions were not completely satisfactory. In practice, there are often difficulties in the etching plant, mainly because of the formation of a coarse grain in the metal. Moreover, the addition of most of the earlier proposed elements is detrimental as to the leakage current and the shelf life of the capacitor.

In the course of long and systematic researches in laboratories and in etching plants we invented an aluminum foil the composition of which not only allows an extraordinary good and uniform etching even without use of electric current, no troubles arising for instance through formation of a coarse grain, but also leads to a great increase of capacity of the electrolytical condensers made from this foil. The increase of capacity amounts to about 20 percent.

The aluminum foil according to our invention is characterized by the fact that it is made from purest aluminum of at least 99.98 percent with the usual amounts of silicon, iron and so on as impurities and contains beside these impurities 0.005 to 0.05 percent boron, 0.001 to 0.005 zinc and 0.0003 to 0.002 percent magnesium, the proportion of zinc to magnesium being greater than 2:1, preferably 3:1 to 4:1. The content of boron, zinc and magnesium has no detrimental influence on the leakage current and the shelf life of the capacitor.

Preferably the iron content is increased, for instance up to 0.006 percent at most. Very good results were obtained with an iron content of 0.003 percent with a tolerance of  $\pm 0.0005$  percent. The increase of the iron content causes a substantial acceleration of the etching. In a hydrochloric acid etching bath, without use of electric current, one may for instance obtain the same roughening within 3 minutes as within 5 minutes without increased iron content.

2

The best results were obtained with a boron content of 0.01 percent with a tolerance of  $\pm 0.005$  percent.

The boron content for itself allows an increase of capacity of the electrolytical condenser by about 20 percent.

However, the addition of boron alone to high purity aluminum does not hinder with certainty the formation of the coarse grain structure.

A content of zinc and magnesium without boron causes a fine grain structure but no appreciable increase of the capacity of the condenser. The highest effect is obtained only with the combined content of boron, zinc and magnesium.

The aluminum foil according to our invention presents for the chemical etching several advantages: one obtains a higher roughening, the etching is shortened and the metal has a fine grain structure. A fine grain structure is important for the rolling as well as for the etching. The advantages appear for instance from the following table:

20

| 25 | Type of high purity aluminum                                   | Electrical values for 540 Volt formation voltage    |                                    | Remarks                                            |
|----|----------------------------------------------------------------|-----------------------------------------------------|------------------------------------|----------------------------------------------------|
|    |                                                                | Capacity of the condenser, $\mu F/100 \text{ cm}^2$ | Surface increase by etching (fold) |                                                    |
| 30 | 99.99 p.c. Al.....                                             | 13-14.5                                             | 5.2-5.8                            | Partly useless because of coarse grain structures. |
|    | 99.99 p.c. Al + 0.0015 p.c. Mg + 0.004 p.c. Zn                 | 14.3-15                                             | 5.7-6.0                            | Throughout fine grain structure.                   |
|    | 99.99 p.c. Al + 0.0025 p.c. B                                  | 15.4                                                | 6.15                               | Partly useless because of coarse grain structure.  |
| 35 | 99.99 p.c. Al + 0.011 p.c. B                                   | 17.1                                                | 6.85                               | Do.                                                |
|    | 99.99 p.c. Al + 0.015 p.c. B + 0.0015 p.c. Mg + 0.0035 p.c. Zn | 18.5                                                | 7.2                                | Throughout fine grain structure.                   |

40

The etching has been carried out according to the method described in Example 2 of the U.S. Patent No. 2,699,382. The foil thickness was 0.1 mm.

45 What we claim is:

1. An aluminum foil for electrolytic condensers of a composition consisting essentially of aluminum, zinc, and magnesium, the aluminum being of a purity not less than 99.98%, the zinc and magnesium being present in amounts sufficient to improve the fineness of the grain structure of the composition, the amount of zinc not exceeding about 0.005% and the amount of magnesium not exceeding about 0.002%.
2. The foil of claim 1 in which the composition contains iron in amount not exceeding about 0.006%.
3. The foil of claim 1 containing also boron in an amount not exceeding 0.05%.
4. The foil of claim 1 wherein the zinc content is between .001 and .005% and the magnesium content between .0003 and .002% with the proportion of zinc to magnesium between 2:1 and 4:1.
5. The foil of claim 2 wherein the iron content is 0.003% with a tolerance of  $\pm 0.0005$ %.
6. The foil of claim 2, the boron content of which is 0.01% with a tolerance of  $\pm 0.0005$ %.
7. The foil of claim 3 wherein the zinc content is between .001 and .005% and the magnesium content between .003 and .002% with the proportion of zinc to magnesium between 2:1 and 4:1.

## References Cited in the file of this patent

## UNITED STATES PATENTS

|           |                |               |
|-----------|----------------|---------------|
| 1,921,998 | Bonsack        | Aug. 8, 1933  |
| 2,252,421 | Stroup         | Aug. 12, 1941 |
| 2,545,866 | Whitzel et al. | Mar. 20, 1951 |

## FOREIGN PATENTS

|         |               |               |
|---------|---------------|---------------|
| 551,872 | Great Britain | Mar. 12, 1943 |
| 552,972 | Great Britain | May 3, 1943   |
| 734,524 | Great Britain | Aug. 3, 1955  |

## OTHER REFERENCES

ASM Transactions, vol. 41, 1949, page 444.

Study on Formation of Dielectric Film of Super-Purity Aluminum Anode in Electrolytic Condensers, 3rd Report, by Nakamura and Nishizaka. Light Metals (Japan), No. 20, 58-67, August 1956. Digested in: Light Metals Bulletin, vol. 19, No. 3, February 1, 1957, page 104.

UNITED STATES PATENT OFFICE  
CERTIFICATE OF CORRECTION

Patent No. 2,886,432

May 12, 1959

Hans Schmitt et al.

It is hereby certified that error appears in the printed specification of the above numbered patent requiring correction and that the said Letters Patent should read as corrected below.

Column 2, line 69, for ".003" read -- .0003 ---.

Signed and sealed this 29th day of September 1959.

(SEAL)

Attest:

KARL H. AXLINE  
Attesting Officer

ROBERT C. WATSON  
Commissioner of Patents